

## UNITED STATES PATENT OFFICE

2,217,805

## PRINTING CELLULOSIC TEXTILE MATERIALS

Denys Percival Milburn, Blackley, Manchester, England, assignor to Imperial Chemical Industries Limited, a corporation of Great Britain

No Drawing. Application March 8, 1938, Serial No. 194,703. In Great Britain March 10, 1937

## 6 Claims. (CL. 8—65)

The present invention relates to the printing of cellulosic textile fabrics in resist styles so that there are produced white patterns on a coloured ground or, alternatively, coloured patterns on a differently coloured ground.

According to the invention cellulosic textile materials are printed with a printing paste containing, besides other usual ingredients, a compound of the general formula

10 R—NCO

where R is an aliphatic hydrocarbon radical having not less than 12 carbon atoms.

The so-printed material is then dried and heated as by steaming for a short time and is then dyed, conveniently by padding; finally, the ground colour having been developed if necessary, the material is washed, soaped and dried in the usual way.

20 It will be understood that when the printing paste contains only the resisting agent, together with the usual thickeners, for example, gum sene-gal, gum tragacanth or British gum, and assistants, for example, emulsifying agents, such as sulphated fatty alcohols, there are produced, finally, white patterns on a coloured ground.

Alternatively the printing paste may contain, in addition to the resist agent and other ingredients, an ice colour preparation which is capable 30 of being developed by treatment with acid. In this case, the steaming operation to which, after printing and drying, the fabric is subjected, is modified in that it is carried out in the presence of the vapour of a suitable acid, for example, 35 formic acid or acetic acid. In this way there are finally produced coloured patterns on a differently coloured ground.

As dyestuffs for providing the ground colour, which is preferably applied by padding I may use 40 vat dyestuffs (applied either as such from reduction medium or in the soluble leuco ester form), azoic colours (applied, for instance, as ready-for-printing preparations of e. g., diazoamino compound and coupling component) or mordant dye-stuffs.

45 In carrying the invention into practical effect it is preferable to work as far as possible at low temperatures (e. g., room temperature), as by using cold padding liquors and drying the fabric after padding by means of hot air rather than by passing it over heated cylinders. It is believed that the success of the process depends upon the production, during the steaming operation, of temporarily water-repellent areas on the fabric where the printing paste has been applied. Such water-repellency would be impaired or destroyed by working at elevated temperatures.

Padding is preferably done through the nip so

as to minimise the time of contact of the fabric with the padding liquor.

Where the resist agent is an isocyanate it is conveniently employed in the form of an aqueous emulsion or suspension which may be produced, if desired, with the aid of an emulsifying agent such, for example, as a sulphated fatty alcohol.

5 As compounds of formula R—NCO suitable to be used in the process of the invention there may be mentioned, for example, dodecyl, tridecyl, tetradecyl, pentadecyl, cetyl, heptadecyl, octadecyl, eicosyl and octadecenyl isocyanates, likewise mixtures of isocyanates such as may be obtained from the mixed amines derived from the mixed acids obtained from coconut oil or stearin.

10 If desired, the said isocyanates may be used in conjunction with other known resist agents, for example gelatine, glue size, or other proteins or albumenoids.

15 As thickening agents there may be used, for example, British gum, starch-British gum, gum Senegal or gum arabic.

The invention is illustrated but not limited by the following examples in which the parts are by weight.

## Example 1

Cotton fabric is printed with a paste made by incorporating together

|                                  | Parts | Parts |
|----------------------------------|-------|-------|
| Heptadecyl isocyanate            | 4     | 30    |
| Sodium cetyl sulphate            | 0.2   |       |
| Starch-tragacanth thickening 1:1 | 50    |       |
| Water                            | 45.8  |       |
|                                  | 100   | 35    |

The printed fabric is dried, steamed for 15 minutes and then grounded by padding in one of the following solutions:

|                                                                                    | A       | B     |
|------------------------------------------------------------------------------------|---------|-------|
| Soledon Jade Green XS paste (the sulphuric ester of leuco dimethoxydibenzanthrone) | Parts 3 | Parts |
| Soledon Orange R powder (Schultz Farbstoffabellen, 7th edn. No. 1349)              | 5       | 1.5   |
| Tragacanth thickening 1:1                                                          | 3       | 5     |
| Sodium nitrite 30% aqueous solution                                                | 89      | 3     |
| Water                                                                              | 100     | 90.5  |
|                                                                                    | 100     | 100   |

40 It is then dried, developed by passing through a 2% solution of sulphuric acid (168° Tw.) at 70° C., washed, soaped and dried. There is thus obtained a clear-cut white pattern on either a green or an orange ground.

## Example 2

50 Cotton fabric is printed and steamed as in

Example 1. It is then grounded by padding in one of the following solutions:

|                                                    | A     | B     |
|----------------------------------------------------|-------|-------|
|                                                    | Parts | Parts |
| 5 Caledon Jade Green paste (Colour Index No. 1101) | 3     | ----- |
| Caledon Blue 3G paste (Colour Index No. 1109)      | 2     | ----- |
| Tragacanth thickening 1:1                          | 5     | 5     |
| Sodium formaldehyde sulphoxylate                   | 6     | 6     |
| Potassium carbonate                                | 12    | 12    |
| 10 Water                                           | 74    | 75    |
|                                                    | 100   | 100   |

The grounded print is dried, steamed for 10 minutes, oxidised in the usual manner to develop the ground colour, soaped at the boil and again dried. There is thus obtained a clear-cut white pattern on either a green or a blue ground.

Example 3

20 Cotton fabric is printed and steamed as in Example 1 and then padded with the following:

|                                                                                                                        | Parts |
|------------------------------------------------------------------------------------------------------------------------|-------|
| 25 A blue dyestuff which is the sodium salt of 1-sulphohydroxydimethylfuchson dicarboxylic acid (Colour Index No. 722) | 1     |
| Acetate of chrome liquor 28° Tw                                                                                        | 7     |
| Tragacanth thickening 1:1                                                                                              | 5     |
| Water                                                                                                                  | 87    |
|                                                                                                                        | 100   |

The grounded print is steamed for 1/2-1 hour, washed, soaped and dried. A clear-cut white pattern on a blue ground is thus obtained.

Example 4

40 Cotton fabric is printed and steamed as in Example 1 and is then padded with one of the following solutions:

|                                                                                                                                                                                                                 | A     | B     |
|-----------------------------------------------------------------------------------------------------------------------------------------------------------------------------------------------------------------|-------|-------|
|                                                                                                                                                                                                                 | Parts | Parts |
| 45 An azoic dyestuff printing preparation as commercially supplied, comprising a mixture of a diazoimino compound of diazotised 4-chloro-o-toluidine and the o-toluidide of 2:3-hydroxy-naphthoic acid          | 0.7   | ----- |
| An azoic dyestuff printing preparation as commercially supplied, comprising a diazoimino compound from diazotised 4-benzoylamino-2:5-dihydroxy-naphthidine mixed with the anilide of 2:3-hydroxy-naphthoic acid | ----- | 1     |
| 50 Caustic soda aqueous solution 76° Tw                                                                                                                                                                         | 1     | 2     |
| Tragacanth thickening 1:1                                                                                                                                                                                       | 5     | 5     |
| Water                                                                                                                                                                                                           | 98.3  | 92    |
|                                                                                                                                                                                                                 | 100   | 100   |

55 It is then dried, steamed for 15 minutes in the presence of acetic and formic acid vapours, washed, soaped at the boil and dried. There is thus obtained a clear-cut white pattern on either a red or a blue ground.

60 Example 5

Cotton fabric is printed and steamed as in Example 1 and is padded in the following liquor:

|                                                                | A  | Parts |
|----------------------------------------------------------------|----|-------|
| 65 Caledon Jade Green X 200 paste fine (Colour Index No. 1101) | 2  | ----- |
| Caustic soda aqueous solution 76° Tw                           | 2  | ----- |
| Sodium hydrosulphite                                           | 2  | ----- |
| 70 Water                                                       | 30 | ----- |
|                                                                | 64 | ----- |
| Water                                                          | 75 | 100   |

A is heated until the dyestuff is completely vatted; it is then cooled and B is added to it.

After padding, the material is exposed to the air for 1/2 minute to develop the dyestuff, then washed, chromed, soaped at the boil and dried. There is obtained a clear-cut white pattern on a green ground.

Example 6

The following mixtures P and Q are made up separately by warming the ingredients together until all is dissolved:

|                                                                                                                                                                                                       | A     | B     |
|-------------------------------------------------------------------------------------------------------------------------------------------------------------------------------------------------------|-------|-------|
|                                                                                                                                                                                                       | Parts | Parts |
| An azoic dyestuff printing preparation, as commercially supplied, comprising a mixture of a diazoimino compound of diazotised 4-chloro-o-toluidine and the o-phenetidine of 2:3-hydroxynaphthoic acid | 7     | ----- |
| An azoic dyestuff printing preparation, as commercially supplied, comprising a mixture of a diazoimino compound of diazotised 4-chloro-o-toluidine and the o-toluidide of 2:3-hydroxynaphthoic acid   | ----- | 20    |
| Methylated spirit                                                                                                                                                                                     | 3     | 3     |
| Aqueous sodium hydroxide 76° Tw                                                                                                                                                                       | 3     | 3     |
| Starch-tragacanth thickening (1:1)                                                                                                                                                                    | 50    | 50    |
| Water                                                                                                                                                                                                 | 15    | 15    |
| (Heptadecyl) isocyanate                                                                                                                                                                               | 4     | 4     |
| Q: Sodium cetyl sulphate                                                                                                                                                                              | 0.2   | 0.2   |
| Water                                                                                                                                                                                                 | 19.8  | 19.8  |
|                                                                                                                                                                                                       | 100   | 100   |

P and Q are then cooled and mixed together to form a printing paste. Cotton fabric is printed with one of the printing pastes A and B. It is then dried and steamed for 15 minutes in the presence of acetic and formic acid vapours. The printed fabric is then grounded by padding in one of the following liquors, solution A being used on material printed with paste A and solution B on material printed with paste B:

|                                                                                                                                            | A     | B     |
|--------------------------------------------------------------------------------------------------------------------------------------------|-------|-------|
|                                                                                                                                            | Parts | Parts |
| Soledon Jade Green XS paste (the sulphuric ester of leuco dimethoxy dibenzanthrone)                                                        | 3     | ----- |
| A blue dyestuff which is the sulphuric ester of leuco 16:17-diethylene ether of dihydroxydibenzanthrone in the form of a 20% aqueous paste | ----- | 45    |
| Tragacanth thickening (1:1)                                                                                                                | 5     | 5     |
| Sodium nitrite 30% aqueous solution                                                                                                        | 3     | 4     |
| Water                                                                                                                                      | 80    | 88    |
|                                                                                                                                            | 100   | 100   |

50 It is then dried, preferably by hot air, and developed by passage through a 2% aqueous solution of sulphuric acid (168° Tw.) at 70° C. It is finally washed, soaped at the boil and dried. There is thus obtained a clear-cut scarlet pattern on a green ground and a clear-cut red pattern on a blue ground.

Example 7

55 Cotton fabric is printed and steamed as in Example 6. It is then grounded by padding with the following liquor:

|                                                                                                                                                                                                              | Parts |
|--------------------------------------------------------------------------------------------------------------------------------------------------------------------------------------------------------------|-------|
| An azoic dyestuff printing preparation as commercially supplied, comprising a mixture of a diazoimino compound of diazotised 4-benzoylamino-2:5-diethoxyaniline and the anilide of 2:3-hydroxynaphthoic acid | 65    |
| Aqueous sodium hydroxide 76° Tw                                                                                                                                                                              | 3     |
| Tragacanth thickening (1:1)                                                                                                                                                                                  | 5     |
| Water                                                                                                                                                                                                        | 90    |
|                                                                                                                                                                                                              | 100   |

It is then dried and steamed in the presence of acetic and formic acid vapours for 1/4 to 1/2 hour.

The material is finally soaped at the boil and dried. There is thus obtained a clear-cut scarlet or red pattern on a blue ground.

Example 8

5 Cotton fabric is printed and steamed as in Example 6. It is then grounded by padding in the following liquor:

|                                                                                                 | Parts |
|-------------------------------------------------------------------------------------------------|-------|
| 10 A blue dyestuff which is the sodium salt of 1-sulphohydroxydimethylfuchson dicarboxylic acid | 1     |
| Aqueous acetate of chrome solution 28° Tw                                                       | 7     |
| Tragacanth thickening (1:1)                                                                     | 5     |
| 15 Water                                                                                        | 87    |
|                                                                                                 | 100   |

20 The printed and grounded fabric is then steamed for  $\frac{1}{2}$  to 1 hour, soaped and dried. There is thus obtained a clear-cut scarlet or red pattern on a blue ground.

Example 9

25 Cotton fabric is printed and steamed as in Example 6. It is then grounded by padding in the following liquor:

|                                            | Parts |
|--------------------------------------------|-------|
| Fast Printing Green S (Colour Index No. 2) | 2     |
| Water                                      | 89    |
| 30 Tragacanth thickening (1:1)             | 5     |
| Aqueous ferrous sulphate 21° Tw            | 4     |
|                                            | 100   |

35 The printed and grounded fabric is then dried and passed through a boiling 1% aqueous solution of sodium carbonate (anhyd.), washed, soaped at the boil and dried. There is obtained a clear-cut scarlet or red pattern on a green ground.

Example 10

40 Cotton fabric is printed and steamed as in Example 6. It is then grounded by padding in the following liquor:

|                                        | Parts |
|----------------------------------------|-------|
| 45 Caledon Jade Green X 200 paste fine | 2     |
| Aqueous caustic soda 76° Tw            | 2     |
| Sodium hydrosulphite                   | 2     |
| Water                                  | 94    |
|                                        | 100   |

50 In making this solution the first three ingredients are heated with 30 parts of water until the dyestuff is completely vatted. The solution is

then cooled and the remaining 64 parts of water are added.

After grounding the material is exposed to the air for  $\frac{1}{2}$  minute to develop the ground colour and is then washed, chromed, soaped at the boil and dried. There is obtained a clear-cut scarlet or red pattern on a green ground.

If in the above examples the heptadecylisocyanate is replaced by an equal weight of hexadecyl isocyanate or octadecylisocyanate, similar excellent resists are obtained.

The above examples deal only with the application of the process to cotton fabric, but it is to be understood that it can be applied also to other cellulosic material, e. g., viscose rayon and also to fabrics constituted in part of other textile fibres, for example certain cotton-wool, viscose-wool or viscose-pure silk unions.

I claim:

1. A process of printing cellulosic textile materials in resist styles to produce patterns on a colored ground which comprises applying to the cellulosic textile material a resist printing paste which contains as the active resist agent an aliphatic isocyanate having the general formula,  $R-NCO$ , where  $R$  is an aliphatic hydrocarbon radical containing 12 or more carbon atoms, drying the material, steaming the material, and then dyeing it to produce a ground shade.

2. A process as claimed in claim 1 wherein the printing paste also contains an ice color preparation capable of being developed by acid.

3. A process as claimed in claim 1 wherein the dyestuff which is used to produce the ground shade is applied by padding.

4. A process as claimed in claim 1 wherein the dyestuff used to provide the ground shade is selected from the group consisting of vat dyestuffs, azoic colors, and mordant dyestuffs.

5. A process of coloring cellulosic fabric in predetermined designs, which comprises printing upon the same in predetermined designs a resist paste comprising as active resist an alkyl isocyanate wherein the alkyl group contains not less than 12 carbon atoms; drying the printed fabric, steaming the dried fabric to develop a temporary water-repellent effect in the printed areas, then padding the fabric with a developable ground color, and further treating the same to develop the ground color.

6. A process as set forth in claim 5 wherein heptadecyl isocyanate is used as the active resist agent in the resist printing paste.

DENYS PERCIVAL MILBURN.